

H. S. EVANS.

METHOD OF DECORATING GLASSWARE.

APPLICATION FILED AUG. 25, 1914.

1,226,957.

Patented May 22, 1917.

2 SHEETS—SHEET 1.



Fig. 2



Fig. 1

WITNESSES

Julian H. Hendig,  
M. L. Jones

INVENTOR

Howard S. Evans

ATTORNEYS

Symmetrist, Bradley, Lechner & Hawkes

1,226,957.

H. S. EVANS.  
METHOD OF DECORATING GLASSWARE.  
APPLICATION FILED AUG. 25, 1914.

Patented May 22, 1917.  
2 SHEETS—SHEET 2.

Fig. 4



Fig. 5



WITNESSES

Julian H. Koenig  
M. L. Jones

INVENTOR

*by* Howard S. Evans  
Symmes, Bradley, Lechner & Fawke

ATTORNEYS

# UNITED STATES PATENT OFFICE.

HOWARD S. EVANS, OF PITTSBURGH, PENNSYLVANIA, ASSIGNOR TO MACBETH-EVANS  
GLASS COMPANY, OF PITTSBURGH, PENNSYLVANIA, A CORPORATION OF PENNSYLVANIA.

## METHOD OF DECORATING GLASSWARE.

1,226,957.

Specification of Letters Patent.

Patented May 22, 1917.

Application filed August 25, 1914. Serial No. 858,443.

To all whom it may concern:

Be it known that I, HOWARD S. EVANS, a citizen of the United States, residing at Pittsburgh, in the county of Allegheny and State of Pennsylvania, have invented certain new and useful Improvements in the Method of Decorating Glassware, of which the following is a specification.

The invention relates to a method for producing colored designs upon glassware and particularly upon shades for use in lighting. The invention has for its objects the provision of a method capable of producing a design of improved appearance; and the provision of a method which can be carried on rapidly and by the exercise of only a slight degree of skill on the part of the operators, so that the cost of the decorating in colors is reduced to a minimum. The method is illustrated in the accompanying drawings wherein—

Figures 1, 2, 3 and 4 are side elevations of shades in successive stages incident to the practice of the method.

Fig. 1 illustrates a shade 1 of clear or other glass, before the process of decoration has begun. This shade is placed in a device for rotating it about its axis and the bands of color 2 and 3 are applied by means of a brush or by a spray. These bands of color might be applied by some other procedure than the one just mentioned, but this method is a rapid and convenient one. After the colors have been dried or burned to fix them upon the glass, the next step of the method, as illustrated in Fig. 3, is practised.

The step, as illustrated in Fig. 3, consists in imprinting upon the bands of color 2 and 3, the designs 4 and 5, such designs being imprinted with a material known in the art as resist. This resist is a relatively sticky substance preferably composed of zinc, rubber cement, and a fat oil of turpentine. This material constitutes a protecting coating so that when a sand blast or other roughening agent is subsequently applied to the shade the surface covered by the resist is protected from the action of the sand blast or roughening agent. In some cases it may be desirable to use in place of the resist a coating or covering consisting of a plate in the form of the design to be produced.

Fig. 4 illustrates the shade after the last 55 steps of the operation. To bring the shade

to this condition, the shade of Fig. 3 is exposed to a sand blast which sand blast not only roughens the surface of the glass not covered by the paint or the resist, but also removes the portion of the painted coating 60 not covered by the resist. The sand blast of course roughens the surface from which the paint has been removed so that the entire surface of the shade with the exception of the design portions 4 and 5, is sanded or 65 roughened. This operation leaves the resist upon the surface of the shade and this resist is then washed away, preferably by means of a soda water solution. The washing away of the resist exposes the colored 70 surface underneath so that the surface of the shade is decorated with a colored design imposed upon polished glass with a sanded background surrounding the colored portions. If desired the process might be, of 75 course, practised in the reverse manner so as to make the portions 4 and 5 constitute the sanded background with the remainder of the shade in colors upon the polished glass. The coloring may or may not be 80 burned. In those cases where the colors are to be burned, this is preferably done after the application of the bands of color as illustrated in Fig. 2, but if desired the burning operation could be deferred until 85 after the sand blasting operation and after the washing off of the resist. Other roughening agents may be employed in place of the sand blast, such as an acid.

The result achieved by the process is advantageous not only because of the unusual appearance secured due to the fact that the colors are imposed upon unsanded glass with a sanded surrounding portion or background therefor, but because of the cheapness of the operation. Very little skill is required to apply the bands of color as illustrated in Fig. 2 or to apply the printed design of resist as illustrated in Fig. 3, the latter operation being accomplished by 100 means of a strip or sheet carrying the resist in the desired design or pattern.

These operations can therefore be carried on with the exercise of only a small amount of care and with great rapidity. The expensive hand labor incident to filling in designs outlined upon the glass surfaces in the manner in which such work has hitherto been done is avoided and the result achieved is better since the colors as applied in the 110

bands 2 and 3, and subsequently appearing in the design, are more uniform than in the procedure above referred to where imprinted outlines are filled in by hand with a brush. The cost of decorating the glass is reduced to a minimum and a product is secured of an appearance better than the more expensive product as heretofore produced. Other advantages incident to the process will be readily apparent to those skilled in the art.

Another manner of carrying out the process is as follows: The glass article is first roughened on the outside, and a dry paint is applied with a piece of cotton or other material to that portion on which the design is to appear. An acid resist is then imprinted on the article upon the colored portion and the article is dipped in acid for a sufficient period to allow it to remove that portion of the colored surface not protected by the resist. This immersion is not continued long enough to permit the acid to etch perceptibly that part of the article not covered by the resist. The resist is then removed, thus finishing the article. The appearance secured with this process is somewhat different than that secured by the process first described, softer and more delicate colors being secured since the roughened surface takes up only a certain amount of the dry paint giving what is known as a matt finish with colors of a relatively subdued tone. If desired the removal of the paint not covered by the resist might be accomplished by means of a sand blast, the resist in that case being of the character described in connection with the first process.

What I claim is:

40 1. The method of producing sanded or ground glassware decorated in colors, which consists in placing upon the articles colored bands, leaving the remainder of the glass uncolored, burning the colors to fix them upon 45 the glass, placing upon the bands protecting coverings of the designs to be produced, treating the articles so that the surfaces thereof with the exception of that which is protected are roughened, and the coloring

matter is removed from the unprotected portions of the bands, and finally removing the said protecting coverings. 50

2. The method of producing sanded or ground glassware decorated in colors, which consists in placing upon the articles colored bands, leaving the rest of the articles uncolored, placing over the bands protecting coverings of the designs to be produced, treating the articles so that the surfaces thereof with the exception of that which is protected 55 are roughened, and the coloring matter is removed from the unprotected portions of the bands, and finally removing the protecting coverings. 60

3. The method of producing sanded or ground glassware decorated in colors, which consists in rotating the articles about their axes and applying colors in bands to the articles as they are rotated, placing over the bands of color produced protecting coverings of the designs to be produced, treating the articles so that the surfaces thereof with the exception of that which is protected are roughened and the coloring matter removed 70 from the unprotected portions, and finally 75 removing the protecting coverings.

4. The method of producing sanded or ground glassware decorated in colors, which consists in coloring portions of the outer surfaces of the articles leaving the remainder 80 of the outer surface of the glass uncolored, burning the colors to fix them upon the glass, placing upon the colored portions protecting coverings of the designs to be produced, treating the articles so that the surfaces thereof with the exception of that which is protected 85 is roughened, and the coloring matter is removed from the unprotected parts of the colored portions, and finally removing the said protecting coverings. 90

In testimony whereof I have hereunto signed my name in the presence of the two subscribed witnesses.

HOWARD S. EVANS.

Witnesses:

ALAN BRIGHT,  
GEORGE D. SHAVER.